

Feb. 27, 1940.

C. L. OCÓN

2,191,972

PRODUCTION OF HIGH QUALITY LUBRICATING OILS BY COLD  
FRACTIONATION, EXTRACTION, AND SYNTHESIS

Filed Nov. 1, 1937



*Cecilio L. Ocón*

INVENTOR.

## UNITED STATES PATENT OFFICE

2,191,972

## PRODUCTION OF HIGH QUALITY LUBRICATING OILS BY COLD FRACTIONATION, EXTRACTION, AND SYNTHESIS

Cecilio L. Océon, Yonkers, N. Y.

Application November 1, 1937, Serial No. 172,088

5 Claims. (Cl. 196—13)

This invention relates particularly to a process for removing from viscous hydrocarbon oils containing desirable lubricating oil constituents, such desirable constituents and constituents having properties which permit improvement to form desirable lubricating oil constituents.

One of the principal objects of this invention is to provide a method for recovering a larger yield of high quality lubricating oil from inferior viscous oils than are obtained only by a solvent extraction of such oils by a solvent or solvents intended to extract selectively aromatic, naphthenic, and unsaturated hydrocarbons which include undesirable lubricating oil constituents. To attain this object, this invention provides, among other things, for a differential separation of valuable constituents removed by the selective solvent extraction, such constituents being highly desirable lubricating oil constituents in spite of their cyclic or unsaturated character and being readily and economically convertible into highly desirable lubricating oil constituents by synthetic treatments described hereinafter.

Another important object of this invention is to provide for a method of synthesizing from the by-products of a cold fractionation and extraction steps, or other processes connected with this process, lubricating constituents which are not only valuable lubricating constituents but which also enhance the lubricating oil product in quality above natural lubricating oils of high quality.

With the above and other objects in view, which will become apparent from a more detailed description following, reference also being made to the self-explanatory schematic flow diagram which illustrates suitable principal steps taken in effecting this invention according to one embodiment.

The starting oil for this process may be any hydrocarbon oil containing the viscous ingredients needed in a lubricating oil used in crank cases of internal combustion engines, such as fractions of crude, mixed base of Mid-Continental crude oils, naphthene base oils, asphalt base oils, or paraffine base oils, especially fractions or residues boiling above 700° F. In the event that such initial oil is an unrefined oil containing undesirable constituents, such as asphaltic and resinous substances, it is first to be refined by using one or more of the following steps: Hydrogenation, distillation, filtration through an absorbent material such as clay, asphalt precipitation, as by means of a low boiling hydrocarbon, or an asphalt absorbent solvent.

The hydrogenation is most suitably one which

is of the type avoiding asphalt formation by use of low temperatures to avoid substantial cracking and dehydrogenation. The distillation is one which is most suitably carried out under vacuum, with the aid of a gaseous distillation agent, or both. The filtration may be carried out in the vapor phase in conjunction with the above described distillation or in the liquid phase with an adsorbent contact agent and other known agents which aid in removing preformed and formative asphaltic substances. The asphalt precipitation can be carried out in well known ways at low temperatures by the addition of normally gaseous constituents in the liquid phase, such as light fractions obtained from stabilizer towers, the precipitated asphaltic material being settled, centrifuged, or filtered from the dissolved oil. In the solvent extraction of the asphaltic material may be used such selective absorbents as liquid sulphur dioxide, aluminum chloride, aniline saturated with water, etc., the absorbent and conditions being adjusted to remove mainly asphaltic and very low viscosity index hydrocarbons.

After the asphalt removal, when necessary, the low asphalt or deasphaltized oil is subjected to a dewaxing, if needed. Some oils will not require the dewaxing and in some instances, such as in the refining with aluminum chloride, it might be found more desirable to remove the wax before attempting to remove the asphaltic constituents. Also, in using the liquefied normally gaseous hydrocarbons or similar wax precipitants it has been found desirable to first remove resinous and asphaltic materials, which interfere with wax precipitation and which contaminate the wax.

The oil with low wax and asphalt content, such as a dewaxed and deasphaltized oil, as explained, is subjected to a selective solvent extraction by a solvent which extracts mainly cyclic and unsaturated hydrocarbons to produce a raffinate of high viscosity index, such solvents as liquid sulphur dioxide, aniline, nitro-hydrocarbons, halogen-hydrocarbons, phenol, etc., being used, either alone, with one another or in mixtures with solubility enhancing agents, such as anthracene, benzene, turpentine, acetone, etc.

The wax constituents removed in a dewaxing step are conveniently employed through a wax treatment to produce an auxiliary solvent for the differential extraction of constituents desirable in a lubricating oil and susceptible to improvement. This wax treatment consists in an improvement involving mainly a splitting of the wax into normally liquid aliphatic molecules in-

cluding isomerization or polymerization into isoparaffins. Primarily, this treatment is a pyrolytic splitting of the wax at low cracking temperatures to avoid the formation of large amounts of naphtha. This can be accomplished by a slow heat treatment of the wax at temperatures between about 800 to 900° F., under a superatmospheric pressure of about 5 to 20 atmospheres or more, for a period of about 60 minutes or longer. Hydrogen or an inert gas may be used to aid in obtaining the pressure and preventing drastic cracking. With extension of time the products can be made to polymerize and isomerize. To shorten the time of treatment the wax may be made to distill over a condensing agent or dehydrating catalyst. It is considered that the wax treatment should mainly produce aliphatic hydrocarbons boiling above 400° F., and largely composed of isoparaffins and monoolefins as well as paraffins. Such hydrocarbons as these have been found useful in the process of the present invention as auxiliary solvents in the differential separation, which is next to be described.

25 The differential separation or differential solvent extraction in this invention is intended to separate from low viscosity index oils, such as, ordinary selective solvent extracts, constituents which are highly valuable present in lubricating oils and those which can readily be transformed into valuable lubricating oil constituents. This object is achieved by the use of a solvent medium which tends to dissolve aliphatic, alkylated cyclic hydrocarbons, and substances of similar nature. 30 Such media comprise low boiling organic liquids of low polarity such as carbon tetra-chloride, higher alcohols such as amyl alcohol or isobutanyl oil (synthetic higher alcohols from reduction of carbon monoxide), alcohol esters, and such media diluted with gasoline hydrocarbons of paraffinic character. To supplement the action of such media it has been found helpful to use a mutually soluble high boiling normally liquid aliphatic compound such as is obtained by 35 the wax treatment described above, or similar oils such as hydrogenated aliphatic polymers produced by the hydrogenation of polymers from gum forming constituents in gasoline and kerosene fraction vapors from a cracking process. 40 This auxiliary solvent of aliphatic character works well if it has a boiling range of about 400 to 650° F., that is, about the boiling range of kerosene and gas oil. It appears that this auxiliary solvent acts to aid the solution of aliphatic or alkylated compounds by virtue of their dispersion effect and non-polar area effect. The 45 recovered oils form the extract in the solution with the medium or solvent and auxiliary solvent. The undissolved or rejected oil, which is believed to be largely polycyclic, e. g., with three or more rings to a molecule, is commercially valuable for forming resins. It is believed that this differential separation is aided not only by the kind of auxiliary solvent described but also by 50 the preliminary step of the deasphalting.

55 The dissolved desirable lubricating constituents may be removed from the differential solvent extract solution by distillation and be added directly to the raffinate from the selective solvent extraction to enhance the recovered lubricating oil without further treatment, or the solution may be subjected to a treatment for synthesizing improved lubricating oil constituents. In using a solvent such as carbon tetra-chloride, which 60 remains more or less inert or at least not detri-

mental to the synthesizing treatment, such a medium need not be removed from the extract from the differential separation for it is even beneficial as a diluent. The synthesizing treatment for improving the differential extracted constituents along with the auxiliary solvent constituents consists in a reaction of such constituents to cause further alkylation of the extracted constituents and polymerization of aliphatics in the auxiliary solvent. This treatment 10 may be accomplished by subjecting the extract solution from the differential separation including such a medium as carbon tetrachloride to the action of aluminum chloride or a similar Friedel-Crafts condensation agent, or to such an 15 agent with the aid of a promoter, such as a hydrogen halide. This may be accomplished by halogenating part of the treated wax products before they are added to the differential separation zone. Such a condensation treatment is 20 carried out at about a temperature of 150 to 300° F., with about 3 to 10% of catalyst on the basis of the material treated.

25 The differentially extracted lubricating constituents or the treated differentially separated constituents, after being separated from the extraction medium and constituents of too low boiling point by distillation, may be added to the raffinate separated from the selective solvent to enhance its quantity and quality or to some other 30 lubricating oil to do the same.

35 As a specific example, a Mid-Continent crude lubricating stock of viscosity index between 75 and 85 is first deasphaltized by treatment with liquid sulphur dioxide added in an amount of about one third the weight of the oil treated, after mixing at a temperature of about 30° F., the mixture being allowed to stratify. An extract of very low viscosity index is removed. The deasphaltized oil is mixed with a butane-propane 40 fraction from a stabilizer tower and cooled to about 10° F., to cause separation of wax, which is filtered off. The dewaxed oil separated from volatiles, is cooled and mixed with about an equal weight of aniline at about 30° F., for selective 45 solvent extraction. Wax obtained by the dewaxing of the sulphur dioxide treated oil is distilled at about 850° F., under a pressure of 15 atmospheres to collect a wax distillate boiling between about 400 and 600° F. The vapors from 50 the still are passed together with a small amount of steam and oxygen over a catalyst made up of pumice impregnated with phosphoric acid and dehydrated. The aniline is removed from the extract and the extract is mixed with hydrocarbons of the treated wax distillate in about equal 55 proportion and with a similar proportion of carbon tetrachloride. Following thorough admixture of these liquids, a separation of the carbon tetrachloride solution at about 40° F. is made. The carbon tetrachloride solution is then admixed with about 5 per cent of its weight of anhydrous aluminum chloride and brought to a 60 temperature of 200° F., hydrogen chloride being passed into the reaction mixture. After about 10 hours of treatment, separation is made by vacuum distillation of a lubricating oil fraction, having a high viscosity index in the neighborhood of 100 or above, and this lubricating fraction is added to aniline raffinate after it is separated from dissolved aniline.

65 With a low asphalt containing hydrogenated or clay treated lubricating oil stock, the sulphur dioxide deasphalting may be dispensed with. In place of the butane-propane dewaxing agent, 70

other agents such as ethylene dichloride may be used. In the wax treatment dehydrating catalysts such as activated alumina, clay or thoria, may be used. Or, in place of using the hydrating-dehydrating step to accelerate the wax treatment, a halogenating-dehalogenating, or simply a halogenating action may be used, such as is obtained by injecting chlorine into the wax undergoing splitting and passing the vapor over a metal such as aluminum, zinc, etc. It is to be understood that numerous other modifications are possible in the practical operation of this process without departing from the scope thereof. For example, it is contemplated that solvent media may be recycled, that fractions of the hydrocarbons lower boiling than the desired lubricating oil fraction from the differential extract or its treated product may be recycled to the differential solvent extraction.

This process is designed to produce lubricating oils with remarkable tenacity or adherence to metal surfaces beside suitable characteristics of viscosity, viscosity-temperature coefficient, low sludge and residual carbon content, low pour point, and other proper qualities for a lubricating oil.

Although the present invention has been described with specific details, it is to be understood that such details are not intended to limit the invention, except in so far as set forth in the accompanying claims.

Having described my invention, what I claim and desire to secure by Letters Patent, is as follows:

1. The method of recovering high quality lubricating oils from inferior lubricating oil stocks which comprises subjecting a lubricating oil stock to a deasphaltizing process, dewaxing such oil which has been deasphaltized, selectively sep-

arating from such deasphaltized and dewaxed oil a relatively more paraffinic fraction, by extracting the relatively less paraffinic constituents, subjecting such extracted constituents to a differential separation by means of normally liquid aliphatic hydrocarbons boiling above 400° F. mixed with a solvent medium for alkyl compounds which differentially extracts desirable lubricating oil constituents of cyclic and unsaturated character but having alkyl side chains which make said constituents soluble in said solvent medium.

2. A process for obtaining high quality lubricating oils from inferior lubricating stocks substantially free of asphalt and wax, which comprises subjecting said lubricating oil stock to a selective solvent extraction by a solvent which extracts the relatively low quality constituents of the oil, subjecting extracted constituents from said selective extraction to a differential separation by aliphatic compounds derived by splitting wax hydrocarbons and a mutually soluble solvent to dissolve out constituents which are desirable as lubricating constituents and which are capable on transformation of forming lubricating constituents by alkylation.

3. A process as in claim 2, in which the mutually soluble solvent is carbon tetrachloride.

4. A process as in claim 2, in which aliphatic compounds used in the differential separation are derived from a distillate fraction higher boiling than gasoline obtained by a splitting of wax molecules.

5. A process as in claim 2, in which the solution from the differential separation is subjected to a treatment with a condensing catalyst to cause alkylation of constituents differentially separated from the selective solvent extract.

CECILIO L. OCÓN.